

# United States Patent Office.

FREDERICK BRAUN AND AUGUSTUS THEODORE SCHMIDT, OF PITTSBURG,  
PENNSYLVANIA.

Letters Patent No. 102,760, dated May 10, 1870.

## IMPROVEMENT IN BLEACHING, TANNING, AND COLORING SPONGES.

The Schedule referred to in these Letters Patent and making part of the same.

To all whom it may concern:

Be it known that we, FREDERICK BRAUN and AUGUSTUS THEODORE SCHMIDT, of Pittsburg, in the county of Allegheny and State of Pennsylvania, have invented a new and useful Improvement in Process for Bleaching, Tanning, and Coloring Sponges; and we do hereby declare the following to be a full, clear, and exact description thereof.

The bleaching of sponges by means of acids has been heretofore practiced, but with the result of injuring the fiber or tissue to such an extent as greatly to impair their value.

By our improvement, we not only remove, in a great degree, the dark coloring matter from the sponge, but also strengthen the tissue to such an extent that it cannot easily be torn, and will last much longer, and this without rendering it harsh or unpleasant to the touch.

We are also enabled to impart a beautiful and delicate permanent color to the sponge, after it has been bleached by the removal of the natural coloring matter.

To enable others skilled in the art to use our improvement, we will proceed to explain the processes employed by us to accomplish the results indicated.

The sponges to be treated, which may be the American sponge, or the sponges from Mediterranean sea, or any other quality of sponge, are first cleansed of sand, coral, and other mechanical impurities or foreign matters, in the usual well-known way of cleaning them; they are then subjected successively to three distinct processes, viz:

First, bleaching or decolorization; second, tanning; third, coloring.

These processes we will describe separately in the order above indicated.

For the purpose of removing the natural dark coloring matter from the sponges, we use a wash, composed of a solution in the proportions of about one ounce of permanganate of potash and one ounce of sulphate of soda, dissolved in from one and a half to two gallons of water, the water being slightly warm, (say, about 90° Fahrenheit,) so as to effect the solution. In place of the permanganate of potash, the permanganate of soda may be employed, and for the sulphate of soda, the sulphate of any of the alkalies may be substituted, if desired, in suitable proportions. Of such solution, one gallon is ordinarily sufficient for every pound of sponges to be treated, but some sponges will require more, and others less than the proportionate quantity of washing solution named, according to their color and quality.

The sponges, cleaned of foreign matters and impurities, as before stated, are immersed in this solution

and worked therein by compression and dilation, so as to wash them thoroughly for about half an hour, or until the liquor in which they are washed becomes clear, by reason of the absorption by the sponges of the chemicals which had been held in solution by the water, or until the sponges have absorbed as much as they will take of the permanganate of potash and sulphate of soda. The result of this washing is partially to soften the sponge tissue, and to give a dark brown color to the sponge.

The sponges are then washed rapidly in a bleaching solution, composed of about one ounce of hyposulphite of soda, with about one ounce of sulphuric acid, in two gallons of water. In this solution two ounces of muriatic acid may be substituted for the one ounce of sulphuric acid.

Washing the sponges, previously treated as before described, in this solution of hyposulphite of soda and sulphuric acid immediately discharges the coloring matter from the sponges, and leaves them nearly colorless.

They are not left in this solution, but are taken out quickly, and then well washed in pure water, and if a more perfect decolorization is desired, the washing in the permanganate of potash solution, and the subsequent dipping in the hyposulphite of soda solution may be repeated, after which they are again rinsed in pure water.

In place of using the wash of hyposulphite of soda and sulphuric or muriatic acid, as above stated, a bath of liquid sulphurous acid may be employed, or the sponges may be exposed to the fumes of sulphurous acid, produced by the combustion of sulphur.

The second process is that of tanning the sponges, which have been bleached as above stated. For this purpose, we use a solution in three gallons of water, of three ounces of muriate of soda (common salt) and nine ounces of sulphate of alumina. In this liquor the sponges are immersed for about twenty-four hours, or until they have rendered the liquor nearly neutral.

They are then removed and dried without being rinsed or washed in pure water, which would tend to remove the tanning liquor.

In place of the tanning liquor above mentioned, may be substituted a solution in the proportion of one ounce of tannin, dissolved in three gallons of water, or a decoction in water of any herb, bark, or root containing tannin may be employed, using such quantities as will give an equivalent proportion of tannin.

The effect of thus tanning the sponge is to strengthen the sponge tissue to such an extent as to render it almost untearable, without rendering it harsh and disagreeable, or injuring its property of absorbing fluids.

If it is desired to communicate a delicate, uniform, and permanent color to the sponge after the bleaching and tanning processes are finished, we resort to the third or coloring process. This consists in dipping the sponges for a moment in an aqueous solution of aqua ammonia (hartshorn.) The strength of this solution determines the depth of color given to the sponge, and will therefore vary accordingly.

A solution of the strength of one ounce of aqua ammonia in from one to two gallons of water will impart a delicate yellow color, which may be deepened to orange color by increasing the quantity of ammonia.

After dipping the sponges in the ammonia solution they are dried without washing, which completes the operation.

The advantages of our improved processes are that the bleaching operation does not injure the texture or tissue of the sponge; that the tanning process adds greatly to its strength, and the coloring process imparts a variety of delicate tints to the sponges, which may be made lighter or darker, as may be desired.

Our mode of treating sponges adds greatly, also, to their commercial value. The common qualities of Florida sponges may thus be made very beautiful and durable, and will command a high price in the market as compared with the same sponges in their natural condition.

Either the tanning or bleaching processes may be used alone, as unbleached sponges may be tanned by our process, or sponges may be bleached by our process, without being subsequently either tanned or colored.

We therefore do not wish to limit our claim of invention to the combination of these processes, which we have described, although when used as we have

described in succession, they produce, as we think, a better and more saleable article.

Nor do we wish to limit ourselves to dyeing sponges with aqua ammonia, because when bleached by means of our process, they may be dyed of various colors by means of many well-known dyes or coloring matter.

What we claim as our invention, and desire to secure by Letters Patent, is—

1. Bleaching or decolorizing sponges by treating them in a solution in water of permanganate of soda or potash and sulphate of soda, or of other alkalies, and subsequently washing them in a solution of hyposulphite of soda or a bath of liquid or gaseous sulphurous acid, substantially as hereinbefore described.

2. Tanning sponges, substantially in the manner as hereinbefore described.

3. Coloring sponges previously bleached, by means of any desired dye or coloring matter.

4. Coloring sponges previously bleached, or bleached and tanned, by dipping them in a solution of aqua ammonia, substantially as described.

5. Sponges bleached and tanned, substantially in the manner hereinbefore described, as a new article of manufacture.

6. Sponges bleached and colored, substantially as hereinbefore described, as a new article of manufacture.

In testimony whereof we, the said FREDERICK BRAUN and AUGUSTUS THEODORE SCHMIDT, have hereunto set our hands.

FREDERICK BRAUN.  
AUGUSTUS T. SCHMIDT.

Witnesses:

JNO. C. NEWMAYER,  
T. B. KERR.